

## UNITED STATES PATENT OFFICE

2,155,349

## ALLOY STEELS

Walther Mathesius and Marcus A. Grossmann,  
Chicago, Ill.; said Grossmann assignor to  
United States Steel Corporation, New York,  
N. Y., a corporation of New Jersey

No Drawing. Original application September  
14, 1935, Serial No. 40,655. Divided and this  
application November 2, 1936, Serial No. 108,899

## 2 Claims. (Cl. 75—126)

The present invention relates to alloy steels.

This application is a division of the application for United States Letters Patent filed on September 14, 1935, by the present applicants, for improvements in Alloy steels, which application 5 bears Serial No. 40,655.

In the strict sense, steel may be said to be an alloy of iron and carbon. However, in a metallurgical sense, in which the term is used in this specification, an alloy steel is steel (that is—iron 10 and carbon) alloyed with another chemical element or other chemical elements.

An object of the present invention is to produce an alloy steel which is well adapted to resist failure by fatigue, especially for use in highly stressed parts, such as springs.

A further object is to produce an alloy steel for general purposes which involves no special equipment in its manufacture and which has improved characteristics over steel as heretofore 20 known and used.

A further object is to provide a steel well adapted for use in cushioning springs, which steel will effectually resist deterioration in service.

25 A further object is to provide an alloy steel in which the characteristics of vanadium are utilized to advantage in the manufacture of alloy steels.

30 A further object is to provide an improved steel well adapted to meet the needs of commercial operation.

Further objects will appear as the description proceeds.

The present invention contemplates the accomplishment of the objects above referred to by providing a shallow hardening alloy steel. To the skilled steel manufacturer the term "shallow hardening alloy steel" has a definite significance, meaning a steel which, when heated to above its 35 critical temperature and then cooled, has a relatively pronounced tendency to change rapidly from the austenitic to the pearlitic type of internal structure. Steel of fine grain structure tends to be shallow hardening, though of course certain alloy steels, even though they be fine grained, may not be shallow hardening in comparison with the steels for which invention is claimed herein. Of course it is possible to produce shallow hardening steel by using a very restricted amount of carbon, and such steel has its uses in the arts. The present invention is limited to steels in which the carbon content is equal to or greater than .45% by weight.

55 In defining the degree of shallow hardening

contemplated in the present invention it may be observed that certain alloy steels, as for example nickel chromium steel, have characteristics differing from steels contemplated in the present invention. As is well known, alloy steels as ordinarily known to metallurgists will, when heated to a temperature of say 1600 deg. F., form austenite, which is understood by metallurgists to be a solution of carbon in iron. As the steel is cooled from the temperature referred to, the structure changes, and when the steel reaches the neighborhood of about 900 deg. F. there is a tendency to form pearlite, which is a tough substance of low hardness. In the case of most alloy steels as now known and used, as for example the nickel chromium steel above referred to, the length of time in the temperature zone in the neighborhood of 900 deg. F. required for the formation of pearlite is in the neighborhood of 20 seconds. The temperature zone referred to 10 may range from 1050 to 850 deg. F. In the case 15 of the alloy steels forming the subject matter of the present invention, the period of time required in the 900 deg. zone referred to is in the neighborhood of 8 seconds. Considering a body 20 of steel which has been heated to say about 1600 deg. F. and quenched in water, it will be readily understood that in the case of nickel chromium steel or the like the period of dwell in the 900 deg. zone referred to may be too short to form 25 pearlite, but said period of dwell may be ample for the formation of pearlite in the composition of shallow hardening steels. In other words, using the example above referred to, the period 30 of time in which the center of the member under 35 test is in the temperature zone of 900 deg. F. above referred to may be less than 20 seconds but more than 8 seconds. In the event that pearlite has not formed in the quenching operation, the alloy steel, upon further cooling, will 40 form martensite, which is a hard material. In the event that pearlite has formed in the center of the member under test in the quenching operation, this pearlite will retain its identity when the member under test has cooled to atmospheric 45 temperature. The above example illustrates a measure which may be applied to define the degree of hardenability contemplated in the present invention. For convenience, the measure of 50 hardenability may be expressed in connection with an alloy steel bar. The present invention contemplates a composition of alloy steel such that when a cylindrical bar of 1½ inches or more in diameter of homogeneous composition 55 is heated to a temperature of approximately

- 1600 deg. F. and then quenched in still water at room temperature, the material at the axis of said bar will, upon cooling to room temperature, have a Rockwell hardness of not more than 5 50—C. Expressed in another way, and referring to the quenching of the alloy steel in oil, the present invention contemplates a composition of alloy steel such that when a cylindrical bar of 1 inch or more in diameter of homogeneous composition is heated to a temperature of approximately 1600 deg. F. and then quenched in still oil at room temperature, the material at the axis of said bar will have a Rockwell hardness of not more than 50—C.
- 15 It will be understood, of course, that the references immediately above made to bars of specified diameters are merely for convenience of definition of one property of these steels. The steels, of course, are useful in members of all 20 dimensions including small sections in which the steels harden through to their axes or midsections.

In carrying out the present invention it is contemplated to use in the manufacture of the improved alloy steel a predominating amount of vanadium either with or without other shallow hardening elements. Correspondingly, the present invention contemplates a relatively low amount of the deep hardening elements (such for 30 example as manganese, chromium and/or nickel). The relative terms referred to in the preceding sentence have reference to the functions of the alloying elements referred to as commonly used in alloy steels in common use today.

35 Proceeding to a more specific definition of alloying elements contemplated in the present invention, the following observations may be made:

Since vanadium reaches its full effectiveness 40 at approximately .15%—.2% by weight, a predominating amount of vanadium in the alloy steel according to the present invention would be approximately .075%—.2% by weight.

On the other hand, chromium may be said to 45 have its greatest effectiveness at about 1.5% by weight, so that a predominating amount of chromium would be about .75%—1.5%.

Since manganese reaches its maximum effectiveness at about 2% by weight, a predominating 50 amount of manganese would be about 1.25%—2% by weight.

Since nickel reaches its full effectiveness at about 3% to 4%, a predominating amount of nickel would be about 1%—4% by weight.

55 Therefore, expressing the purpose of the present invention in other language, it may be said that the present invention contemplates the use of vanadium in the amount of .075%—.2% by weight, said element being used without chromium or manganese if preferred; or, if chromium be used, then with less than .75% by weight of chromium; or, if manganese be used, then with less than 1.25% of manganese. Expressed in still other language, certain advantages of the present invention will be had if the shallow hardening element (vanadium) is used to a percentage equal to at least 50% of its fully effective amount in opposing hardening in quenched steels; and certain advantages of the present invention will be 60 had if the deep hardening elements (for example chromium, manganese and/or nickel) are restricted to not more than 50% of their fully effective amounts as hardening agents in quenched steels. Another way of defining the limits of the 70 materials contemplated in the present invention

is by reference to the "critical cooling rate" of the materials. Critical cooling rate of steels may be defined as that rate above which a steel will harden in the cooling process and below which a steel will not harden. When the term "harden" is used in this connection it is intended to convey the meaning that the material of the steel becomes the hard material "martensite." The present invention contemplates steels which when quenched in a quenching medium at atmospheric temperatures will just harden if it passes 1325 deg. F. at a rate above 50 deg. per second but below 150 deg. per second.

Those skilled in the art will understand that manganese is usually present in the manufacture of steel to the extent of about .2%—.5% by weight, since manganese is commonly used as a de-oxidizer in steel making; and for the same reason silicon is usually present in amounts of about .2%.

Proceeding now to a still more specific recitation of analysis of steel falling within the scope of the present invention, the following example may be recited:

|                | Per cent    | 25 |
|----------------|-------------|----|
| Carbon from    | .85 to .95  |    |
| Manganese from | .20 to .50  |    |
| Silicon from   | .10 to .35  |    |
| Chromium from  | .20 to .50  |    |
| Vanadium from  | .075 to .20 | 30 |

Balance largely iron with traces of impurities.

It will be understood, of course, that the analysis above noted is illustrative only, and the objects of the present invention may be realized by proper balancing of shallow hardening elements against deep hardening elements. For example, the carbon may vary from .30% to 1%; the manganese may vary from .40% to 1.25%; the chromium may vary from 0 to .75%; the vanadium may vary from .075% to .20%. A choice 40 of the elements referred to to provide a shallow hardening steel meeting the tests recited in this specification will fall within the scope of this invention.

45 Anyone familiar with the manufacture of alloy steels has readily available to him information as to the constituents and the amounts thereof which must be used in producing the steels having the foregoing analyses.

In arriving at the object of making a shallow hardening alloy steel, the present invention contemplates a steel of fine grain size. In referring to fine grain size it is to be understood that reference is had to the grain size of austenite, which is the structure composing the steel when the steel has been heated to a high temperature (for example 1600 deg. F.) preparatory to hardening by quenching. The term "fine grain" or "fine grain size" as used in this specification means 55 from #5 to #8 on the ASTM chart of grain sizes. This may be further explained as meaning more than 12 grains per square inch when examined at a magnification of 100 diameters.

60 The fact is well known that fine grain size tends to shallow hardening. It is also well known that very fine grains, particularly #7 and #8, according to the ASTM chart, exhibit structural features known as abnormality, meaning thereby a particular distribution of the iron carbide (that is—cementite) observed in the carburizing test (McQuaid-Ehn carburizing test), which test is used in determining grain size.

65 As is well known, the usual method of discovering the austenite grain size of the steel is to car- 70

burize said steel at about 1700 deg. F. for about eight hours. The carbon absorbed in this carburizing operation will upon cooling arrange itself at the boundaries of the austenite grains and so outline them, thus making it possible to determine the size of these austenite grains. In coarse-grained steels this carbon (which is usually present in the form of iron carbide or cementite) arranges itself in continuous layers or envelopes which completely and clearly outline the austenite grains. In very fine-grained steels, however, the iron carbide coalesces into separate particles, so that the grain boundaries are not outlined continuously. This latter condition of the iron carbide (cementite), associated with a small amount of ferrite in its immediate neighborhood, is often termed divorce of the iron carbide or cementite and is commonly known as abnormality. Divorce of the cementite or iron carbide has been referred to by some as dispersion of the cementite.

In order to arrive at fine grain size (including abnormality) it has been common to add, in the furnace ladle or in the molds, about one pound of aluminum per ton of steel. It has been discovered that if vanadium be used as one of the shallow hardening elements, the amount of aluminum may be materially reduced. Vanadium tends to produce fine grain structure and shallow hardening in steel over a relatively wide temperature range in the hardening operation.

The alloy steels forming the subject matter of this invention are characterized by a high degree of ductility, toughness, resiliency and resistance to shock and fatigue.

As is well known, silicon is used in the manufacture of alloy quality steels for the purpose of combining with the oxygen and thereby removing said oxygen. An excess of silicon always appears

in the finished steel of this type and may properly be considered to be a trace of impurity. According to the appended claims such silicon will be included under the term "traces of impurities."

Though certain preferred analyses and steps have been recited in the foregoing specification, many modifications will occur to those skilled in the art. It is intended to cover all such modifications that fall within the scope of the appended claims.

What is claimed is—

1. A shallow hardening alloy steel which is composed of the following ingredients substantially in the amounts specified:

|                 | Per cent    |
|-----------------|-------------|
| Carbon from—    | .85 to .95  |
| Manganese from— | .20 to .50  |
| Chromium from—  | .20 to .50  |
| Vanadium from—  | .075 to .20 |

balance iron with traces of impurities, said steel being characterized by a high degree of ductility, toughness, resiliency and resistance to shock and fatigue.

2. An alloy steel characterized by a high degree of resilience and resistance to shock and fatigue which is composed of the following ingredients within the ranges specified and balanced against each other to produce a shallow hardening steel:

|                 | Per cent                     |
|-----------------|------------------------------|
| Carbon from—    | .45 to 1                     |
| Manganese from— | .40 to 1.25                  |
| Chromium from—  | an appreciable amount to .75 |
| Vanadium from—  | .075 to .20                  |

remainder iron with traces of impurities.

WALTHER MATHESIUS.  
MARCUS A. GROSSMANN.

CERTIFICATE OF CORRECTION.

Patent No. 2,155,349.

April 18, 1939.

WALTHER MATHESIUS, ET AL.

It is hereby certified that error appears in the printed specification of the above numbered patent requiring correction as follows: Page 2, second column, line 26, for "95" read .95; page 3, first column, line 37, for the word "allow" read alloy; and that the said Letters Patent should be read with this correction therein that the same may conform to the record of the case in the Patent Office.

Signed and sealed this 13th day of June, A. D. 1939.

(Seal)

Acting Commissioner of Patents.